

July 10, 1923.

1,461,347

H. E. COOK

CARRIAGE FULL BAND FOR TYPEWRITING AND LIKE MACHINES

Filed Sept. 24, 1920



WITNESSES

Lillian Nelson.

*Charles O. Smith*

INVENTOR  
Harry E. Cook  
By Jacob Feltel  
HIS ATTORNEY

## UNITED STATES PATENT OFFICE.

HARRY E. COOK, OF WASHINGTON, DISTRICT OF COLUMBIA, ASSIGNOR TO REMINGTON TYPEWRITER COMPANY, OF ILION, NEW YORK, A CORPORATION OF NEW YORK.

## CARRIAGE PULL BAND FOR TYPEWRITING AND LIKE MACHINES.

Application filed September 24, 1920. Serial No. 412,426.

To all whom it may concern:

Be it known that I, HARRY E. Cook, citizen of the United States, and resident of the city of Washington, District of Columbia, have invented certain new and useful Improvements in Carriage Pull Bands for Typewriting and like Machines, of which the following is a specification.

My invention relates to pull bands for typewriting and like machines.

It has been customary heretofore to use metallic and textile pull or draw bands to connect the carriage of a typewriting or like machine to its spring drum or motor in order to move the carriage from the motor through said pull band. Certain disadvantages have been found in the use of both metallic and textile pull bands formerly employed. While metallic bands possess certain advantages over the textile bands, the former are liable in the operation of the machine to slip off the drum of the motor on which they are wound and become buckled, twisted or damaged. The textile bands also are liable to slip off the drum, and the lack of stiffness in the textile bands render them more difficult to connect with the drum or carriage than the stiffer metallic bands. This difficulty is more pronounced and time consuming in some machines than in others, as where, for example, the band must be threaded around or through parts of the machine to make the connection.

The main object of my invention, generally stated, is to overcome these defects and provide a simple, effective and inexpensive pull band which will not readily slip from the surface of the motor drum on which it is wound, and which nevertheless is stiff enough to be readily threaded through or around parts of the machine and be connected to the motor drum and carriage.

To the above and other ends which will hereinafter appear, my invention consists in a pull band of the character set forth in the following description and particularly pointed out in the appended claim.

In the accompanying drawings wherein like reference characters indicate corresponding parts in the various views,

Figure 1 is an enlarged detail face view of a textile pull band of the usual construc-

tion before it is treated in the manner to be 65 hereinafter described.

Figure 2 is a fragmentary edge view of the same.

Figure 3 is an edge view of the same pull band after having been treated. 60

Figure 4 is a fragmentary face view of the same.

The band as shown in Fig. 1 comprises a textile body portion or strip of suitable woven fabric 1, such for example as is now 65 in common use. To each end of the strip is shown attached a fastening device 2 by which the band is connected at one end to the spring drum and at the other end to the carriage. In the present instance a free end of the strip is passed through an opening 3 in one of the devices 2 and is bent back on itself to form a loop around a cross bar 4 of the fastening device. The free end of the strip is then connected to the body 70 portion thereof by a sheet metal clamp or clip 5, which presses and holds the contacting parts of the band together. 75

In treating the textile band in accordance with my invention I incorporate therein a stiffening substance which preferably is likewise sufficiently adhesive to prevent the band from easily slipping off the spring drum on which it is wound. Good results have been obtained by the use of a glutinous substance 80 such as rosin. One method of treatment which has produced a band that is highly effective in use is the following:—A textile band of the character described, and such as is shown in Fig. 1, is placed in a bath or compound composed of three parts rosin and one part alcohol by bulk. After it has remained in the compound about fifteen minutes the band is removed and held at its 85 ends by two supports in a taut condition to prevent it from shrinking. The band is held in this condition until it is air-dried sufficiently to be in a condition for use, 90

which generally requires about twelve hours. The proportions of rosin and alcohol employed may be varied. A test to determine 95 how far these proportions may be varied is to press the substance between the fingers. When the substance becomes sticky it may be used effectively.

It will be understood that by treating the band in the manner described, the outstanding fibres (which I have attempted to show

in Figs. 1 and 2) sink and become more closely incorporated in the body of the band as shown in Figs. 3 and 4. The compound also serves to connect the fibres together adhesively, thus adding strength to the band without in any manner injuring the fibres but, on the other hand, adding to the durability thereof. The band after being treated and dried in the manner described will be comparatively stiff, though flexible, corresponding approximately to the stiffness and flexibility of a metal band, which enables it to be easily threaded into the machine and readily connected to the spring drum and carriage. Moreover, the substance used to stiffen the band is of such a character that the band has a strong tendency to cling to the smooth surface of the drum on which it is wound, thus avoiding the hitherto ob-

jectionable liability of readily slipping off the drum.

What I claim as new and desire to secure by Letters Patent, is:—

A pull band for typewriting and like machines, the body portion of which is made wholly of textile material and has rosin incorporated in its otherwise untreated body sufficient in quantity to render the band stiff enough to thread through parts of a machine and clingy enough to prevent slipping.

Signed at the city of Washington, District of Columbia, this 20th day of September, A. D. 1920.

HARRY E. COOK.

Witnesses:

W. J. McNALLY,  
JNO. T. MEANY.